



US006150082A

# United States Patent [19]

Nakamura et al.

[11] Patent Number: 6,150,082

[45] Date of Patent: Nov. 21, 2000

[54] SILVER HALIDE PHOTOGRAPHIC MATERIAL

[75] Inventors: Tetsuo Nakamura; Ryuji Abe; Takanori Hioki, all of Kanagawa, Japan

[73] Assignee: Fuji Photo Film Co., Ltd., Kanagawa, Japan

[21] Appl. No.: 09/170,075

[22] Filed: Oct. 13, 1998

## [30] Foreign Application Priority Data

Oct. 14, 1997 [JP] Japan ..... 9-280938

[51] Int. Cl.<sup>7</sup> ..... G03C 1/18; G03C 1/34

[52] U.S. Cl. ..... 430/574; 430/572; 430/585; 430/611

[58] Field of Search ..... 430/585, 611, 430/574, 572

## [56] References Cited

## U.S. PATENT DOCUMENTS

4,791,053 12/1988 Ogawa ..... 430/581  
5,290,673 3/1994 Nishikawa ..... 430/567  
5,534,403 7/1996 Nishigaki et al. ..... 430/585

Primary Examiner—Thorl Chea

Attorney, Agent, or Firm—Sughrue, Mion, Zinn, Macpeak &amp; Seas, PLLC

[57]

## ABSTRACT

A silver halide photographic material is disclosed which contains at least one compound represented by the following formula (I) and at least one dye having the absorption maximum in a methanol solution at from 510 to 535 nm:



wherein R<sup>1</sup> and R<sup>2</sup> each represents an alkyl group; Y represents an aryl group or a heterocyclic group; V<sup>1</sup>, V<sup>2</sup>, V<sup>3</sup> and V<sup>4</sup> each represents a hydrogen atom, a halogen atom, an alkyl group, an alkoxy group, a hydroxyl group, an alkylthio group, a mercapto group, a cyano group, an acyl group, a carboxyl group, or an alkoxy carbonyl group; X<sup>1</sup> represents a counter ion; and m<sup>1</sup> represents a number of 0 or more necessary for neutralizing a charge in the molecule.

6 Claims, No Drawings

## SILVER HALIDE PHOTOGRAPHIC MATERIAL

## FIELD OF THE INVENTION

The present invention relates to a silver halide photographic material, and more specifically relates to a silver halide photographic material which is high sensitive, generates less fog, exhibits excellent storage stability and excellent graininess.

## BACKGROUND OF THE INVENTION

Every endeavor has been made for higher sensitization and improvement of graininess of a silver halide photographic material. It is known that a sensitizing dye which is used for spectral sensitization largely affects capacities of a silver halide photographic material. A trace of structural difference of a sensitizing dye largely affects photographic capacities such as sensitivity, fog, storage stability and graininess, and the combined use of two or more sensitizing dyes also greatly influences photographic capacities, but it is difficult to foresee its effect. Many engineers have hitherto synthesized various kinds of sensitizing dyes, have examined combinations of a variety of sensitizing dyes and have endeavored to investigate photographic capacities thereby, but it is not possible to know photographic capacities in advance yet.

From the above reasons, techniques of spectrally sensitizing silver halide grains (in particular, reduction sensitized silver halide grains) high sensitively without causing malefic effects such as generation of fog and deterioration of graininess have been demanded.

On the other hand, a trial of reduction sensitization for higher sensitization of a silver halide photographic material has been studied heretofore. Various compounds are disclosed in many patents as useful reduction sensitizers, for example, tin compounds are disclosed in U.S. Pat. No. 2,487,850, polyamine compounds in U.S. Pat. No. 2,512,925, and thiourea dioxide compounds in British Patent 789,823. Further, in *Photographic Science and Engineering*, Vol. 23, p. 113 (1979), comparisons of natures of silver nuclei formed according to various reduction sensitizing methods are described and dimethylamineborane, stannous chloride, hydrazine, and methods of high pH ripening and low pAg ripening have been employed. Reduction sensitizing methods are also disclosed in U.S. Pat. Nos. 2,518,698, 3,201,254, 3,411,917, 3,779,777 and 3,930,867. Not only the selection of reduction sensitizers but contrivances of reduction sensitizing methods are disclosed in JP-B-57-33572 and JP-B-58-1410 (the term "JP-B" as used herein means an "examined Japanese patent publication").

## SUMMARY OF THE INVENTION

An object of the present invention is to provide a silver halide photographic material which is high sensitive, generates less fog, is excellent in storage stability and excellent in graininess.

As a result of eager investigations, the above object of the present invention has been attained by the following means.

(1) A silver halide photographic material which comprises at least one compound represented by the following formula (I) and at least one dye having the absorption maximum in a methanol solution at from 510 to 535 nm:



wherein R<sup>1</sup> and R<sup>2</sup> each represents an alkyl group; Y represents an aryl group or a heterocyclic group; V<sup>1</sup>, V<sup>2</sup>, V<sup>3</sup> and V<sup>4</sup> each represents a hydrogen atom, a halogen atom, an alkyl group, an alkoxy group, a hydroxyl group, an alkylthio group, a mercapto group, a cyano group, an acyl group, a carboxyl group, or an alkoxy carbonyl group; X<sup>1</sup> represents a counter ion; and m<sup>1</sup> represents a number of 0 or more necessary for neutralizing a charge in the molecule.

(2) The silver halide photographic material as described in (1), wherein the compound represented by formula (I) is represented by the following formula (II):



wherein R<sup>11</sup> and R<sup>12</sup> each represents an alkyl group; W<sup>1</sup>, W<sup>2</sup>, W<sup>3</sup>, W<sup>4</sup> and W<sup>5</sup> each represents a hydrogen atom or a substituent; V<sup>11</sup> and V<sup>12</sup> each represents a hydrogen atom or a halogen atom; X<sup>2</sup> represents a counter ion; and m<sup>2</sup> represents a number of 0 or more necessary for neutralizing a charge in the molecule.

(3) The silver halide photographic material as described in (1), which comprises a support having provided thereon at least one silver halide emulsion layer, wherein the silver halide grains of the silver halide emulsion layer are reduction sensitized and the silver halide emulsion layer comprises at least one compound represented by formula (I) and at least one dye having the absorption maximum in a methanol solution at from 510 to 535 nm.

(4) The silver halide photographic material as described in (3), wherein the compound represented by formula (I) is represented by the above formula (II).

(5) The silver halide photographic material as described in (3), wherein the dye having the absorption maximum in a methanol solution at from 510 to 535 nm has the structure represented by the following formula (III), (IV) or (V):



65

wherein R<sup>31</sup> and R<sup>32</sup> each represents an alkyl group; V<sup>31</sup>, V<sup>32</sup>, V<sup>33</sup>, V<sup>34</sup>, V<sup>35</sup>, V<sup>36</sup>, V<sup>37</sup> and V<sup>38</sup> each represents a hydrogen atom or a substituent; Z<sup>3</sup> represents a hydrogen

atom, a methyl group or an ethyl group;  $X^3$  represents a counter ion; and  $m^3$  represents a number of 0 or more necessary for neutralizing a charge in the molecule;



wherein  $R^{41}$  and  $R^{42}$  each represents an alkyl group;  $V^{41}$ ,  $V^{42}$ ,  $V^{43}$ ,  $V^{44}$ ,  $V^{45}$ ,  $V^{46}$ ,  $V^{47}$  and  $V^{48}$  each represents a hydrogen atom or a substituent, provided that any one of the combinations of  $V^{41}$  and  $V^{42}$ ,  $V^{42}$  and  $V^{43}$ , and  $V^{43}$  and  $V^{44}$  link to each other to form a benzo condensed ring, and any one of the combinations of  $V^{45}$  and  $V^{46}$ ,  $V^{46}$  and  $V^{47}$ , and  $V^{47}$  and  $V^{48}$  link to each other to form a benzo condensed ring;  $Z^4$  represents a hydrogen atom, a methyl group or an ethyl group;  $X^4$  represents a counter ion; and  $m^4$  represents a number of 0 or more necessary for neutralizing a charge in the molecule;



wherein  $R^{51}$ ,  $R^{52}$ ,  $R^{53}$  and  $R^{54}$  each represents an alkyl group;  $V^{51}$ ,  $V^{52}$ ,  $V^{53}$ ,  $V^{54}$ ,  $V^{55}$ ,  $V^{56}$ ,  $V^{57}$  and  $V^{58}$  each represents a hydrogen atom or a substituent;  $Z^5$  represents a hydrogen atom, a methyl group or an ethyl group;  $X^5$  represents a counter ion; and  $m^5$  represents a number of 0 or more necessary for neutralizing a charge in the molecule.

(6) The silver halide photographic material as described in (5), wherein the dye having the absorption maximum in a methanol solution at from 510 to 535 nm has the structure represented by formula (III).

(7) The silver halide photographic material as described in any of (1), (2), (3), (4), (5) or (6), wherein the silver halide photographic material contains at least one compound represented by the following formula (VI), (VII) or (VIII):



wherein  $R^{101}$ ,  $R^{102}$  and  $R^{103}$  each represents an aliphatic group, an aromatic group or a heterocyclic group;  $M^{101}$  represents a cation;  $E$  represents a divalent linking group, and  $a$  represents 0 or 1.

#### DETAILED DESCRIPTION OF THE INVENTION

Compounds for use in the present invention are described in detail below.

In formulae (I) and (II), examples of alkyl groups represented by  $R^1$ ,  $R^2$ ,  $R^{11}$  and  $R^{12}$  include an unsubstituted alkyl group having from 1 to 8, preferably from 1 to 4, carbon atoms (e.g., methyl, ethyl, propyl, isopropyl, butyl, isobutyl, hexyl), or a substituted alkyl group having from 1 to 8, preferably from 1 to 4, carbon atoms [substituents thereof include, e.g., a carboxyl group, a sulfo group, a cyano group, a halogen atom (e.g., fluorine, chlorine, bromine, iodine), a hydroxyl group, an alkoxy carbonyl group having from 1 to 7 carbon atoms (e.g., methoxycarbonyl, ethoxycarbonyl, benzyloxycarbonyl), an aryloxycarbonyl group having from 1 to 7 carbon atoms (e.g., phenoxy carbonyl), an alkoxy group having from 1 to 7 carbon atoms (e.g., methoxy, ethoxy, benzyloxy), an aryloxy group having 6 or 7 carbon atoms (e.g., phenoxy, p-tolylloxy), an acyloxy group having from 1 to 7 carbon atoms (e.g., acetoxy, propionyloxy), an acyl group having from 1 to 7 carbon atoms (e.g., acetyl, propionyl, benzoyl), a carbamoyl group (e.g., carbamoyl,  $N,N$ -dimethylcarbamoyl, morpholino carbonyl, piperidinocarbonyl), a sulfamoyl group (e.g., sulfamoyl,  $N,N$ -dimethylsulfamoyl, morpholinosulfonyl, piperidinosulfonyl), an aryl group having from 1 to 7 carbon atoms (e.g., phenyl, p-chlorophenyl, p-tolyl), a sulfonylcarbamoyl group, and an acylsulfamoyl group]. More preferred examples include an alkyl group substituted with a dissociable group such as a carboxyalkyl group (e.g., carboxymethyl, 2-carboxyethyl), an alkane-sulfonylcarbamoylalkyl group (e.g., methanesulfonylcarbamoyl-methyl), and a sulfoalkyl group (e.g., 2-sulfoethyl, 3-sulfo-propyl, 4-sulfobutyl, 3-sulfobutyl), and still more preferred is a sulfoalkyl group. Particularly preferably,  $R^1$  and  $R^{11}$  each represents a 2-sulfoethyl group and  $R^2$  and  $R^{12}$  each represents a 3-sulfopropyl group or a 4-sulfobutyl group.

In formulae (I) and (II), the halogen atoms represented by  $V^1$ ,  $V^2$ ,  $V^3$ ,  $V^4$ ,  $V^{11}$  and  $V^{12}$  are preferably fluorine, chlorine, bromine and iodine, more preferably fluorine and chlorine, and particularly preferably chlorine.

As alkyl groups represented by  $V^1$ ,  $V^2$ ,  $V^3$  and  $V^4$  in formula (I), an alkyl group having from 1 to 4 carbon atoms which may have a substituent (e.g., methyl, ethyl, propyl, butyl, hydroxymethyl, trifluoromethyl) is preferred, and methyl is more preferred.

As alkoxy groups represented by  $V^1$ ,  $V^2$ ,  $V^3$  and  $V^4$  in formula (I), an alkoxy group having from 1 to 4 carbon atoms which may have a substituent (e.g., methoxy, ethoxy, 2-methoxyethoxy) is preferred and methoxy is more preferred.

As alkylthio groups represented by  $V^1$ ,  $V^2$ ,  $V^3$  and  $V^4$  in formula (I), an alkylthio group having from 1 to 4 carbon atoms which may have a substituent (e.g., methylthio, ethylthio) is preferred and methylthio is more preferred.

As acyl groups represented by  $V^1$ ,  $V^2$ ,  $V^3$  and  $V^4$  in formula (I), an acyl group having from 2 to 5 carbon atoms which may have a substituent (e.g., acetyl, trichloroacetyl) is preferred and acetyl is more preferred.

As alkoxy carbonyl groups represented by  $V^1$ ,  $V_2$ ,  $V^3$  and  $V^4$  in formula (I), an alkoxy carbonyl group having from 2 to 5 carbon atoms which may have a substituent (e.g., methoxy carbonyl, ethoxycarbonyl) is preferred and methoxycarbonyl is more preferred.

$V^1$ ,  $V^3$  and  $V^4$  in formula (I) and  $V^{12}$  in formula (II) each more preferably represents a hydrogen atom, and  $V^2$  and  $V^{11}$  each more preferably represents a halogen atom.  $V^2$  and  $V^{11}$  particularly preferably represent a fluorine atom or a chlorine atom.

The aryl group represented by Y in formula (I) is a substituted or unsubstituted aryl group having from 6 to 15, preferably from 6 to 10, carbon atoms (e.g., phenyl, naphthyl, p-carboxyphenyl, p-nitrophenyl, p-chlorophenyl, 3,5-dichlorophenyl, p-bromophenyl, p-cyanophenyl, m-fluoro-phenyl, p-tolyl). The heterocyclic group represented Y in formula (I) is, e.g., a heterocyclic group having from 1 to 20, preferably from 2 to 10, and more preferably from 4 to 6, carbon atoms, which may be substituted (e.g., pyridyl, 5-methylpyridyl, thienyl, furyl, morpholino, tetrahydro-furfuryl). The heterocyclic group may have the structure of the condensation of a benzene ring, a naphthalene ring or an anthracene ring.

Y in formula (I) preferably represents an aryl group, more preferably a substituted or unsubstituted phenyl group, and particularly preferably an unsubstituted phenyl group.

Substituents represented by  $W^1$ ,  $W^2$ ,  $W^3$ ,  $W^4$  and  $W^5$  in formula (II) are not particularly limited and examples of substituents include, for example, a halogen atom (e.g., fluorine, chlorine, bromine, iodine), a mercapto group, a cyano group, a carboxyl group, a sulfo group, a phosphoric acid group, a hydroxyl group, a carbamoyl group having from 1 to 10, preferably from 2 to 8, and more preferably from 2 to 5, carbon atoms (e.g., methylcarbamoyl, ethylcarbamoyl, morpholinocarbonyl), a sulfamoyl group having from 0 to 10, preferably from 2 to 8, and more preferably from 2 to 5, carbon atoms (e.g., methylsulfamoyl, ethylsulfamoyl, piperidinosulfonyl), a nitro group, an alkoxy group having from 1 to 20, preferably from 1 to 10, and more preferably from 1 to 8, carbon atoms (methoxy, ethoxy, 2-methoxyethoxy, phenethoxy), an aryloxy group having from 6 to 20, preferably from 6 to 12, and more preferably from 6 to 10, carbon atoms (e.g., phenoxy, p-tolyloxy, p-chlorophenoxy,  $\alpha$ -naphthoxy), an acyl group having from 1 to 20, preferably from 2 to 12, and more preferably from 2 to 8, carbon atoms (e.g., acetyl, trichloroacetyl, benzoyl), an acyloxy group having from 1 to 20, preferably from 2 to 12, and more preferably from 2 to 8, carbon atoms (e.g., acetyloxy, benzyloxy), an acylamino group having from 1 to 20, preferably from 2 to 12, and more preferably from 2 to 8, carbon atoms (e.g., acetylamino), a sulfonyl group having from 1 to 20, preferably from 1 to 10, and more preferably from 1 to 8, carbon atoms (e.g., methanesulfonyl, ethane-sulfonyl, benzenesulfonyl), a sulfinyl group having from 1 to 20, preferably from 1 to 10, and more preferably from 1 to 8, carbon atoms (e.g., methanesulfinyl, benzenesulfinyl), a sulfonylamino group having from 1 to 20, preferably from 1 to 10, and more preferably from 1 to 8, carbon atoms (e.g., methanesulfonylamino, ethanesulfonylamino, benzenesulfonyl-amino), an amino group, a substituted amino group having from 1 to 20, preferably from 1 to 12, and more preferably from 1 to 8, carbon atoms (e.g., methylamino, dimethylamino, benzyl-amino, anilino, diphenylamino), an ammonium group having from 0 to 15, preferably from 3 to 10, and more preferably from 3 to 6, carbon atoms (e.g., trimethylammonium, triethylammonium), a hydrazino group having from 0 to 15, preferably from 1 to 10, and more preferably from 1 to 6, carbon atoms (e.g., trimethylhydrazino), a ureido group having from 1 to 15, preferably from 1 to 10, and more preferably from 1 to 6, carbon atoms (e.g., N,N-dimethylureido), an imido group having from 1 to 15, preferably from 1 to 10, and more preferably from 1 to 6, carbon atoms (e.g., succinimido), an alkylthio or arylthio group having from 1 to 20, preferably from 1 to 12, and more preferably from 1 to 8, carbon atoms (e.g., methylthio, ethylthio, carboxyethylthio, sulfobutyl-thio, phenylthio), an alkoxy-carbonyl group having from 2 to 20, preferably from 2 to 12, and more preferably from 2 to 8, carbon atoms (e.g., methoxycarbonyl, ethoxycarbonyl, benzyl-oxy carbonyl), an

aryloxycarbonyl group having from 6 to 20, preferably from 6 to 12, and more preferably from 6 to 8, carbon atoms (e.g., phenoxy carbonyl), an unsubstituted alkyl group having from 1 to 18, preferably from 1 to 10, and more preferably from 1 to 5, carbon atoms (e.g., methyl, ethyl, propyl, butyl), a substituted alkyl group having from 1 to 18, preferably from 1 to 10, and more preferably from 1 to 5, carbon atoms [e.g., hydroxymethyl, trifluoromethyl, benzyl, carboxyethyl, ethoxycarbonylmethyl, acetylaminomethyl, further, an unsaturated hydrocarbon group having from 2 to 18, preferably from 3 to 10, and more preferably from 3 to 5, carbon atoms (e.g., vinyl, ethynyl, 1-cyclohexenyl, benzylidene, benzylidene) is also included in a substituted alkyl group], a substituted or unsubstituted aryl group having from 6 to 20, preferably from 6 to 15, and more preferably from 6 to 10, carbon atoms (e.g., phenyl, p-carboxyphenyl, p-nitrophenyl, 3,5-dichlorophenyl, p-cyano-phenyl, m-fluorophenyl, p-tolyl,  $\alpha$ -naphthyl), and a hetero-cyclic group having from 1 to 20, preferably from 2 to 10, and more preferably from 4 to 6, carbon atoms, which may be substituted (e.g., 2-pyridyl, 2-thienyl, 2-furyl, morpholino, 2-tetrahydrofurfuryl). Two adjacent substituents may be linked to each other to form the structure of condensation of a benzene ring or a naphthalene ring. These substituents may further have a substituent.  $W^1$ ,  $W^2$ ,  $W^3$ ,  $W^4$  and  $W^5$  preferably represent a hydrogen atom.

$X^1$  and  $X^2$  in formulae (I) and (II) are included in the formulae to show the presence of a cation or an anion when a counter ion is necessary for neutralizing an ionic charge in the molecule of the compound. Whether a certain dye is a compound having a cation or an anion or net ionic charge depends on the substituents. Examples of representative cations as a counter ion include inorganic cations such as a hydrogen ion, an alkali metal ion (e.g., a sodium ion, a potassium ion, a lithium ion), and an alkaline earth metal ion (e.g., a calcium ion), and organic cations such as an ammonium ion (e.g., an ammonium ion, a tetraalkylammonium ion, a pyridinium ion, an ethylpyridinium ion). Anions may be either inorganic or organic, and examples include a halide anion (e.g., a fluoride ion, a chloride ion, a bromide ion, an iodide ion), a substituted arylsulfonate ion (e.g., a p-toluenesulfonate ion, a p-chlorobenzenesulfonate ion), an arylsulfonate ion (e.g., a 1,3-benzenedisulfonate ion, a 2,6-naphthalenedisulfonate ion), an alkylsulfate ion (e.g., a methylsulfate ion), a sulfate ion, a thiocyanate ion, a perchlorate ion, a tetrafluoroborate ion, a picrate ion, an acetate ion, and a trifluoromethanesulfonate ion. In addition, ionic polymers or other dyes having a counter charge to the dye can also be used as a counter ion.

Preferred cations are a sodium ion, a potassium ion, a triethylammonium ion, a tetraethylammonium ion, a pyridinium ion, an ethylpyridinium ion, and a methylpyridinium ion. Preferred anions are a perchlorate ion, an iodide ion, a bromide ion, and a substituted arylsulfonate ion (e.g., a p-toluenesulfonate ion).

In the present invention, a sulfo group is described as  $SO_3^-$ , but it can be described as  $SO_3H$  when the compound has a hydrogen ion as a counter ion.

$m^1$  and  $m^2$  each represents a number of 0 or more necessary for balancing a charge in the molecule of the compound and when an inner salt is formed, the number is 0, preferably from 0 to 4.

Specific examples of the compounds represented by formula (I) or (II) according to the present invention are shown below, but it should not be construed as the present invention is limited thereto.

I-1



I-2



I-3



I-4



I-5



I-6



I-7







-continued



II-11



II-12

A sensitizing dye having the absorption maximum in a methanol solution at from 510 to 535 nm which is used in combination with the compound represented by formula (I) or (II) may be a cyanine dye, a merocyanine dye or a composite cyanine dye, preferably a cyanine dye. It is preferred that the absorption maximum in a methanol solution of the sensitizing dye be in the range of from 515 to 530 nm, particularly preferably in the range of from 520 to 530 nm. More preferably, such a sensitizing dye is a compound represented by the following formula (III), (IV) or (V):



In formulae (III), (IV) and (V),  $R^{31}$ ,  $R^{32}$ ,  $R^{41}$ ,  $R^{42}$ ,  $R^{51}$ ,  $R^{52}$ ,  $R^{53}$  and  $R^{54}$  each represents an alkyl group, and as preferred alkyl groups, those cited as preferred alkyl groups for  $R^1$  and  $R^2$  in formula (I) can be exemplified.

In formulae (III), (IV) and (V),  $V^{31}$ ,  $V^{32}$ ,  $V^{33}$ ,  $V^{34}$ ,  $V^{35}$ ,  $V^{36}$ ,  $V^{37}$ ,  $V^{38}$ ,  $V^{41}$ ,  $V^{42}$ ,  $V^{43}$ ,  $V^{44}$ ,  $V^{45}$ ,  $V^{46}$ ,  $V^{47}$ ,  $V^{48}$ ,  $V^{51}$ ,  $V^{52}$ ,  $V^{53}$ ,  $V^{54}$ ,  $V^{55}$ ,  $V^{56}$ ,  $V^{57}$  and  $V^{58}$  each represents a hydrogen atom or a substituent, provided that any of the combinations of  $V^{41}$  and  $V^{42}$ ,  $V^{42}$  and  $V^{43}$ , and  $V^{43}$  and  $V^{44}$  link to each other to form a benzo condensed ring, and any one of the combinations of  $V^{45}$  and  $V^{46}$ ,  $V^{46}$  and  $V^{47}$ , and  $V^{47}$  and  $V^{48}$  link to each other to form a benzo condensed ring in formula (IV). Preferred examples of substituents other than groups which form a benzo condensed ring are the same as those exemplified as preferred substituents for  $W^1$ ,  $W^2$ ,  $W^3$ ,  $W^4$  and  $W^5$ .

In formulae (III), (IV) and (V),  $Z^3$ ,  $Z^4$  and  $Z^5$  each represents a hydrogen atom, a methyl group or an ethyl group, but  $Z^3$  and  $Z^4$  in formulae (III) and (IV) each preferably represents a methyl group or an ethyl group and  $Z^5$  in formula (V) preferably represents a hydrogen atom.

In formulae (III), (IV) and (V),  $X^3$ ,  $X^4$  and  $X^5$  each represents a counter ion, and preferred ions are the same as those exemplified as preferred ions for  $X^1$  and  $X^2$  in formulae (I) and (II).

In formulae (III), (IV) and (V),  $m^3$ ,  $m^4$  and  $m^5$  each represents a number of 0 or more necessary for neutralizing a charge in the molecule and when an inner salt is formed, the number is 0, preferably from 0 to 4.

Specific examples of compounds represented by formula (III), (IV) or (V) are shown below. In particular, the compound represented by formula (III) is preferred.

|       |  |                                       | Maximum Absorption<br>in Methanol Solution |
|-------|--|---------------------------------------|--------------------------------------------|
| III-1 |  | $\text{Na}^+$                         | 525 nm                                     |
| III-2 |  |                                       | 525 nm                                     |
| III-3 |  | $\text{K}^+$                          | 530 nm                                     |
| III-4 |  |                                       | 525 nm                                     |
| III-5 |  | $\text{K}^+$                          | 528 nm                                     |
| III-6 |  | $\text{HN}(\text{C}_2\text{H}_5)_3^+$ | 530 nm                                     |
| IV-1  |  | $\text{Na}^+$                         | 516 nm                                     |
| IV-2  |  |                                       | 516 nm                                     |

-continued

Maximum Absorption  
in Methanol Solution

-continued

|     |                                                                                   | Maximum Absorption<br>in Methanol Solution |
|-----|-----------------------------------------------------------------------------------|--------------------------------------------|
| V-4 |  | 516 nm                                     |
| V-5 |  | 522 nm                                     |

Besides the sensitizing dyes represented by formula (I) or (II) and the sensitizing dyes having the absorption maximum in a methanol solution at from 510 to 535 nm, other sensitizing dyes may also be used in the present invention. Sensitizing dyes are often used in combination, in particular, for the purpose of supersensitization. Representative examples thereof are disclosed in U.S. Pat. Nos. 2,688,545, 2,977,229, 3,397,060, 3,522,052, 3,527,641, 3,617,293, 3,628,964, 3,666,480, 3,672,898, 3,679,428, 3,703,377, 3,769,301, 3,814,609, 3,837,862, 4,026,707, British Patents 1,344,281, 1,507,803, JP-B-43-4936, JP-B-53-12375, and JP-A-52-110618 and JP-A-52-109925 (the term "JP-A" as used herein means an "unexamined published Japanese patent application")

The sensitizing dyes for use in the present invention can be synthesized according to the methods described in the following literature:

- a) F. M. Harmer, *Heterocyclic Compounds—Cyanine Dyes and Related Compounds*, John Wiley & Sons, New York, London (1964)
- b) D. M. Sturmer, *Heterocyclic Compounds—Special Topics in Heterocyclic Chemistry*, Chap. 18, Clause 14, pp. 482 to 515, John Wiley & Sons, New York, London (1977)
- c) *Rodd's Chemistry of Carbon Compounds*, 2nd Ed., Vol. IV, Part B, Chap. 15, pp. 369 to 422, Elsevier Science Publishing Company Inc., New York (1977)

For the inclusion of the sensitizing dyes according to the present invention in the silver halide emulsion of the present invention, they may be directly dispersed in the emulsion, or they may be dissolved in water, a single or mixed solvent of methanol, ethanol, propanol, acetone, methyl cellosolve, 2,2,3,3-tetrafluoropropanol, 2,2,2-trifluoro-ethanol, 3-methoxy-1-propanol, 3-methoxy-1-butanol, 1-methoxy-2-propanol, N,N-dimethylformamide, etc., and then added to the emulsion.

In addition, various methods can be used for the inclusion of sensitizing dyes in the emulsion, for example, a method in which sensitizing dyes are dissolved in a volatile organic

solvent, the solution is dispersed in water or hydrophilic colloid and this dispersion is added to the emulsion as disclosed in U.S. Pat. No. 3,469,987, a method comprising dispersing water-insoluble dyes in a water-soluble solvent without dissolution and adding the dispersion to the emulsion as disclosed in JP-B-46-24185, a method in which dyes are dissolved in acid and the solution is added to the emulsion, or sensitizing dyes are added to the emulsion as an aqueous solution coexisting with acid or base as disclosed in JP-B-44-23389, JP-B-44-27555 and JP-B-57-22091, a method in which dyes are added to the emulsion as an aqueous solution or colloidal dispersion coexisting with a surfactant as disclosed in U.S. Pat. Nos. 3,822,135 and 4,006,026, a method in which dyes are directly dispersed in a hydrophilic colloid and the dispersion is added to the emulsion as disclosed in JP-A-53-102733 and JP-A-58-105141, or a method comprising dissolving dyes using a compound capable of red-shifting and adding the solution to the emulsion as disclosed in JP-A-51-74624 can be used. Further, ultrasonic waves can be used for dissolution.

The time of the addition of the sensitizing dyes according to the present invention to the silver halide emulsion of the present invention may be at any stage of the preparation of the emulsion recognized as useful hitherto. For example, they may be added at any stage if it is before coating, i.e., before grain formation stage of silver halide grains and/or before desalting stage, during desalting stage and/or after desalting and before beginning of chemical sensitization, as disclosed in U.S. Pat. Nos. 2,735,766, 3,628,960, 4,183,756, 4,225,666, JP-A-58-184142 and JP-A-60-196749, or immediately before or during chemical ripening, after chemical ripening and before coating as disclosed in JP-A-58-113920. Also, as disclosed in U.S. Pat. No. 4,225,666 and JP-A-58-7629, the sensitizing dyes can be used as a single compound alone or in combination with compounds having different structures, and they can be divided and added separately, for example, one part of them is added during grain formation stage and the remaining is added during chemical ripening or after the completion of chemical ripening, otherwise one

part is added prior to chemical ripening or during ripening stage and the remaining after completion of chemical sensitization. The kinds of compounds added separately and combinations of compounds may be varied.

Although the use amount of the sensitizing dyes for use in the present invention varies depending on the shapes and the sizes of silver halide grains to be used, but is generally from 0.1 to 4 mmol, preferably from 0.2 to 2.5 mmol, per mol of the silver halide. They may be used in combination with other sensitizing dyes.

The compound represented by formula (I) for use in the present invention is preferably used in an amount of 0.2 to 2.0 mmol/mol-Ag.

The dye having the absorption maximum in a methanol solution for use in the present invention is preferably used in an amount of 0.01 to 5 mmol/mol-Ag.

It is preferred to use an oxidizing agent for silver during the production process of the emulsion of the present invention. An oxidizing agent for silver is a compound having a function of acting on metal silver and converting it to a silver ion. In particular, a compound which can convert superminute silver grains by-produced in the course of the formation of silver halide grains and chemical sensitization to a silver ion is effective. The silver ion converted may form hardly water-soluble silver salt such as silver halide, silver sulfide or silver selenide, or may form easily water-soluble silver salt such as silver nitrate. The oxidizing agent for silver may be inorganic or organic. Examples of inorganic oxidizing agents include ozone, oxyacid salt, such as hydrogen peroxide and addition products thereof (e.g.,  $\text{NaBO}_2 \cdot \text{H}_2\text{O}_2 \cdot 3\text{H}_2\text{O}$ ,  $2\text{Na}_2\text{CO}_3 \cdot 3\text{H}_2\text{O}_2$ ,  $\text{Na}_2\text{P}_2\text{O}_7 \cdot 2\text{H}_2\text{O}_2$ ,  $2\text{Na}_2\text{SO}_4 \cdot \text{H}_2\text{O}_2 \cdot 2\text{H}_2\text{O}$ ), peroxyacid salt (e.g.,  $\text{K}_2\text{S}_2\text{O}_8$ ,  $\text{K}_2\text{C}_2\text{O}_6$ ,  $\text{K}_2\text{P}_2\text{O}_8$ ), a peroxy complex compound (e.g.,  $\text{K}_2[\text{Ti}(\text{O}_2\text{C}_2\text{O}_4)_3\text{H}_2\text{O}_2]$ ,  $4\text{K}_2\text{SO}_4 \cdot \text{Ti}(\text{O}_2\text{OH})\text{SO}_4 \cdot 2\text{H}_2\text{O}$ ,  $\text{Na}_3[\text{VO}(\text{O}_2(\text{C}_2\text{H}_4)_2)_6\text{H}_2\text{O}_2]$ ), permanganate (e.g.,  $\text{KMnO}_4$ ), and chromate (e.g.,  $\text{K}_2\text{Cr}_2\text{O}_7$ ), a halogen element such as iodine and bromine, perhalogen acid salt (e.g., potassium periodate), a metal salt of high valency (e.g., potassium hexacyanoferrate-(III)), and thiosulfonate. Further, examples of organic oxidizing agents include quinones such as p-quinone, an organic peroxide such as peracetic acid and perbenzoic acid, a compound which releases active halogen (e.g., N-bromo-succinimide, chloramine T, chloramine B).

Disulfide compounds disclosed in EP-A-627657 are more preferred oxidizing agents.

The oxidizing agents which are preferably used in the present invention are inorganic oxidizing agents such as ozone, hydrogen peroxide and addition products thereof, a halogen element, and thiosulfinate, and organic oxidizing agents such as quinones. It is preferred to use the above-described reduction sensitization in combination with an oxidizing agent for silver. The method of usage can be selected from a method in which an oxidizing agent is used and then reduction sensitization is carried out, an inverse method thereof, or a method in which both are concurred with. These methods can be used selectively in a grain formation process or in a chemical sensitization process.

The oxidizing agents for use in the present invention may be used in an amount of  $10^{-7}$  to  $10^{-1}$  mol/mol-Ag, preferably  $10^{-6}$  to  $10^{-2}$  mol/mol-Ag, more preferably  $10^{-5}$  to  $10^{-3}$  mol/mol-Ag.

The silver halide photographic material according to the present invention preferably contains at least one compound selected from the compounds represented by formula (VI), (VII) or (VIII).



(VI)



(VI)

(VIII)



wherein  $\text{R}^{101}$ ,  $\text{R}^{102}$  and  $\text{R}^{103}$  each represents an aliphatic group, an aromatic group or a heterocyclic group;  $\text{M}^{101}$  represents a cation;  $\text{E}$  represents a divalent linking group; and  $\text{a}$  represents 0 or 1.

The compounds represented by formula (VI), (VII) and (VIII) are described in detail below.

When  $\text{R}^{101}$ ,  $\text{R}^{102}$  and  $\text{R}^{103}$  each represents an aliphatic group, the aliphatic group is preferably an alkyl group having from 1 to 22 carbon atoms, an alkenyl group having from 2 to 22 carbon atoms, or an alkynyl group having from 2 to 22 carbon atoms, and these groups may be substituted. Examples of alkyl groups include, e.g., methyl, ethyl, propyl, butyl, pentyl, hexyl, octyl, 2-ethylhexyl, decyl, dodecyl, hexadecyl, octadecyl, cyclohexyl, isopropyl and t-butyl.

Examples of alkenyl groups include, e.g., allyl and butenyl.

Examples of alkynyl groups include, e.g., propargyl and butynyl.

When  $\text{R}^{101}$ ,  $\text{R}^{102}$  and  $\text{R}^{103}$  each represents an aromatic group, the aromatic group is preferably an aromatic group having from 6 to 20 carbon atoms, e.g., phenyl and naphthyl. These groups may be substituted.

When  $\text{R}^{101}$ ,  $\text{R}^{102}$  and  $\text{R}^{103}$  each represents a heterocyclic group, the heterocyclic group is a 3 to 15-membered ring having at least one element selected from nitrogen, oxygen, sulfur, selenium and tellurium. Examples of heterocyclic rings include, e.g., a pyrrolidine ring, a piperidine ring, a pyridine ring, a tetrahydrofuran ring, a thiophene ring, an oxazole ring, a thiazole ring, an imidazole ring, a benzothiazole ring, a benzoxazole ring, a benzimidazole ring, a selenazole ring, a benzoselenazole ring, a tellurazole ring, a triazole ring, a benzotriazole ring, a tetrazole ring, an oxadiazole ring, and a thiadiazole ring.

Examples of substituents for  $\text{R}^{101}$ ,  $\text{R}^{102}$  and  $\text{R}^{103}$  include, e.g., an alkyl group (e.g., methyl, ethyl, hexyl), an alkoxy group (e.g., methoxy, ethoxy, octyloxy), an aryl group (e.g., phenyl, naphthyl, tolyl), a hydroxyl group, a halogen atom (e.g., fluorine, chlorine, bromine, iodine), an aryloxy group (e.g., phenoxy), an alkylthio group (e.g., methylthio, butylthio), an arylthio group (e.g., phenylthio), an acyl group (e.g., acetyl, propionyl, butyryl, valeryl), a sulfonyl group (e.g., methanesulfonyl, benzenesulfonyl), an acylamino group (e.g., acetylamino, benzoylamino), a sulfonylamino group (e.g., methanesulfonylamino, benzenesulfonylamino), an acyloxy group (e.g., acetoxy, benzoxy), a carboxyl group, a cyano group, a sulfo group, and an amino group.

$\text{E}$  preferably represents a divalent aliphatic group or a divalent aromatic group. Examples of divalent aliphatic groups represented by  $\text{E}$  include, e.g.,  $-(\text{CH}_2)_n-$  (n is from 1 to 12),  $-\text{CH}_2-\text{CH}=\text{CH}-\text{CH}_2-$ ,



$-\text{CH}_2-\text{C}\equiv\text{C}-\text{CH}_2-$  a xylylene group, etc.

Examples of divalent aromatic groups represented by E include, e.g., phenylene and naphthylene.

M<sup>101</sup> preferably represents a metal ion or an organic cation. Examples of metal ions include a lithium ion, a sodium ion, and a potassium ion. Examples of organic cations include an ammonium ion (e.g., ammonium, tetramethylammonium, tetrabutylammonium), a phosphonium ion (e.g., tetraphenyl-phosphonium), a guanidinium ion, etc.

Specific examples of the compounds represented by formula (VI), (VII) or (VIII) are shown below, but the present invention is not limited to these compounds.

|                                                                                                                                      |         |    |  |
|--------------------------------------------------------------------------------------------------------------------------------------|---------|----|--|
| CH <sub>3</sub> SO <sub>2</sub> SNa                                                                                                  | (VI-1)  | 5  |  |
| C <sub>2</sub> H <sub>5</sub> SO <sub>2</sub> SNa                                                                                    | (VI-2)  | 20 |  |
| C <sub>3</sub> H <sub>7</sub> SO <sub>2</sub> SK                                                                                     | (VI-3)  |    |  |
| C <sub>4</sub> H <sub>9</sub> SO <sub>2</sub> SLi                                                                                    | (VI-4)  | 25 |  |
| C <sub>6</sub> H <sub>13</sub> SO <sub>2</sub> SNa                                                                                   | (VI-5)  |    |  |
| C <sub>8</sub> H <sub>17</sub> SO <sub>2</sub> SNa                                                                                   | (VI-6)  | 30 |  |
| CH <sub>3</sub> (CH <sub>2</sub> ) <sub>3</sub> CHCH <sub>2</sub> SO <sub>2</sub> S•NH <sub>4</sub><br>C <sub>2</sub> H <sub>5</sub> | (VI-7)  |    |  |
| C <sub>10</sub> H <sub>21</sub> SO <sub>2</sub> SNa                                                                                  | (VI-8)  | 35 |  |
| C <sub>12</sub> H <sub>25</sub> SO <sub>2</sub> SNa                                                                                  | (VI-9)  |    |  |
| C <sub>16</sub> H <sub>33</sub> SO <sub>2</sub> SNa                                                                                  | (VI-10) | 40 |  |
| CH <sub>3</sub><br>CH <sub>3</sub> CH—SO <sub>2</sub> SK                                                                             | (VI-11) |    |  |
| t-C <sub>4</sub> H <sub>9</sub> SO <sub>2</sub> SNa                                                                                  | (VI-12) | 45 |  |
| CH <sub>3</sub> OCH <sub>2</sub> CH <sub>2</sub> SO <sub>2</sub> S•Na                                                                | (VI-13) |    |  |
| CH <sub>2</sub> —CHCH <sub>2</sub> SO <sub>2</sub> SNa                                                                               | (VI-14) | 50 |  |
| Cl—  —SO <sub>2</sub> Na                          | (VI-15) | 55 |  |
| Cl—  —SO <sub>2</sub> Na                          | (VI-16) | 60 |  |
|                                                                                                                                      | (VI-17) |    |  |
|                                                                                                                                      | (VI-18) | 65 |  |
|                                                                                                                                      | (VI-19) |    |  |
|                                                                                                                                      | (VI-20) |    |  |
|                                                                                                                                      | (VI-21) |    |  |
|                                                                                                                                      | (VI-22) |    |  |
|                                                                                                                                      | (VI-23) |    |  |
|                                                                                                                                      | (VI-24) |    |  |
|                                                                                                                                      | (VI-25) |    |  |
|                                                                                                                                      | (VI-26) |    |  |
|                                                                                                                                      | (VI-27) |    |  |
|                                                                                                                                      | (VI-28) |    |  |
|                                                                                                                                      | (VI-29) |    |  |
|                                                                                                                                      | (VI-30) |    |  |
|                                                                                                                                      | (VI-31) |    |  |





-continued



(VII-23)



(VII-24)

x/y = 2/1 (mol ratio)

(VII-25)



(VIII-1)



(VIII-2)

C2H5SO2SCH2CH2SO2CH2CH2SSO2C2H5

(VIII-3)



(VIII-4)



(VIII-5)



(VIII-6)



(VIII-7)

C2H5SO2SSSO2C2H5

(VIII-8)

(n)C3H7SO2SSSO2C3H7(n)

(VIII-9)



The compound represented by formula (VI) can be easily synthesized according to the methods disclosed in JP-A-54-1019 and British Patent 972,211.

The compound represented by formula (VI), (VII) or (VIII) is preferably added in an amount of from  $10^{-7}$  to  $10^{-1}$  mol, more preferably from  $10^{-6}$  to  $10^{-2}$  mol, and particularly preferably from  $10^{-5}$  to  $10^{-3}$  mol, per mol of the silver halide.

For adding the compound represented by formula (VI), (VII) or (VIII) to an emulsion during the production process

thereof, methods usually used for adding additives to a photographic emulsion can be used. For example, a compound which is soluble in water is added as an aqueous solution having proper concentration, and a compound which is insoluble or hardly soluble in water is dissolved in an appropriate organic solvent which is miscible with water and does not adversely affect photographic properties selected from alcohols, glycols, ketones, esters or amides, and added as a solution.

10 The compound represented by formula (VI), (VII) or (VIII) can be added to an emulsion at any stage such as during the grain formation of a silver halide emulsion, before or after chemical sensitization. The compound is preferably added before reduction sensitization is conducted 15 or during reduction sensitization is being conducted. The compound is particularly preferably added during grain growing.

The compound may be previously added to a reaction vessel but it is more preferred to be added at an appropriate 20 stage during grain formation. Further, the method comprising previously adding the compound represented by formula (VI), (VII) or (VIII) to an aqueous solution of water-soluble silver salt or an aqueous solution of water-soluble alkali halide and growing grains using these aqueous solutions can 25 be employed. In addition, the solution of the compound represented by formula (VI), (VII) or (VIII) may be divided to several parts and added in several times or may be added continuously over a long period of time with the degree of the grain growth.

30 Of the compounds represented by formula (VI), (VII) or (VIII), the compound represented by formula (VI) is most preferably used in the present invention.

With respect to various techniques and inorganic and 35 organic materials which can be used in the silver halide photographic material according to the present invention, in general, those disclosed in *Research Disclosure*, No. 308119 (1989) and *ibid.*, No. 37038 (1995) can be used.

In addition to these, more specifically, for example, techniques and inorganic and organic materials which can be 40 used in the color photographic material to which the silver halide photographic emulsion of the present invention is applicable are disclosed in the following places of EP-A-436938 and the patents cited in the following places.

45

|     | Item                     | Place                                                                                                                       |
|-----|--------------------------|-----------------------------------------------------------------------------------------------------------------------------|
| 1)  | Layer Structure          | line 34, page 146 to line 25, page 147                                                                                      |
| 2)  | Silver Halide Emulsion   | line 26, page 147 to line 12, page 148                                                                                      |
| 3)  | Yellow Coupler           | line 35, page 137 to line 33, page 146, lines 21 to 23, page 149                                                            |
| 4)  | Magenta Coupler          | lines 24 to 28, page 149; line 5, page 3 to line 55, page 25 of EP-A-421453                                                 |
| 5)  | Cyan Coupler             | lines 29 to 33, page 149; line 28, page 3 to line 2, page 40 of EP-A-432804                                                 |
| 6)  | Polymer Coupler          | lines 34 to 38, page 149; line 39, page 113 to line 37, page 123 of EP-A-435334                                             |
| 7)  | Colored Coupler          | line 42, page 53 to line 34, page 137, lines 39 to 45, page 149                                                             |
| 8)  | Other Functional Coupler | line 1, page 7 to line 41, page 53, line 46, page 149 to line 3 page 150; line 1, page 3 to line 50, page 29 of EP-A-435334 |
| 9)  | Preservative             | lines 25 to 28, page 150                                                                                                    |
| 10) | Formalin                 | lines 15 to 17, page 149                                                                                                    |

-continued

| Item                                            | Place                                                                         |
|-------------------------------------------------|-------------------------------------------------------------------------------|
| Scavenger                                       |                                                                               |
| 11) Other Additives                             | lines 38 to 47, page 153; line 21, page 75 to line 56, page 84 of EP-A-421453 |
| 12) Dispersion Method                           | lines 4 to 24, page 150                                                       |
| 13) Support                                     | line 32 to 34, page 150                                                       |
| 14) Film Thickness, Physical Properties of Film | lines 35 to 49, page 150                                                      |
| 15) Color Development Process                   | line 50, page 150 to line 47, page 151                                        |
| 16) Desilvering Process                         | line 48, page 151 to line 53, page 152                                        |
| 17) Automatic Processor                         | line 54, page 152 to line 2, page 153                                         |
| 18) Washing and Stabilizing Processes           | lines 3 to 37, page 153                                                       |

The silver halide emulsion prepared according to the present invention can be used in color photographic materials, e.g., a color paper, a color film for photographing, and a color reversal film, and black-and-white photographic materials, e.g., an X-ray film, a general film for photographing, and a photographic film for printing.

Exposure methods of silver halide photographic materials according to the present invention are described. Exposure for obtaining photographic images may be performed in usual methods. That is, any of well-known various light sources can be used as exposure light sources, e.g., natural light (sunlight), a tungsten lamp, a fluorescent lamp, a mercury lamp, a xenon arc lamp, a carbon arc lamp, a xenon flash lamp, a laser light, an emission diode, and CRT. Exposure time of shorter than  $1/1,000$  sec., e.g., from  $1/10^4$  to  $1/10^6$  sec. using a xenon flash lamp, and longer than 1 sec. can be used, as well as exposure of from  $1/1,000$  to 1 sec. used in usual cameras. If necessary, spectral composition of the light for use in exposure can be adjusted using a color filter. Exposure can be effected using light emitted from fluorescent materials excited by an electron beam, an X-ray, a  $\gamma$ -ray or an  $\alpha$ -ray.

The present invention will be illustrated in more detail with reference to examples below, but these are not to be construed as limiting the invention.

#### EXAMPLE 1

##### Preparation of Sample No. 101

A multilayer color photographic material was prepared as Sample No. 101 by coating each layer having the following composition on an undercoated cellulose triacetate film support having the thickness of 127  $\mu\text{m}$ . The numeral corresponding to each component indicates the addition amount per  $\text{m}^2$ . The function of the compounds added is not limited to the use described.

-continued

| Second Layer: Interlayer                           |                                           |                |         |
|----------------------------------------------------|-------------------------------------------|----------------|---------|
| 5                                                  | Gelatin                                   | silver amount: | 0.38 g  |
| Compound Cpd-K                                     |                                           |                |         |
|                                                    | Ultraviolet Absorber U-2                  | silver amount: | 5.0 mg  |
|                                                    | High Boiling Point Organic Solvent Oil-3  | silver amount: | 3.0 mg  |
|                                                    | Dye D-4                                   | silver amount: | 0.06 g  |
|                                                    |                                           | silver amount: | 10.0 mg |
| Third Layer: Interlayer                            |                                           |                |         |
| 10                                                 | Yellow Colloidal Silver                   | silver amount: | 0.007 g |
|                                                    | Gelatin                                   | silver amount: | 0.40 g  |
| Fourth Layer: First Red-Sensitive Emulsion Layer   |                                           |                |         |
| 15                                                 | Emulsion A                                | silver amount: | 0.55 g  |
|                                                    | Emulsion B                                | silver amount: | 0.23 g  |
|                                                    | Surface Fogged Fine Grain                 | silver amount: | 0.07 g  |
|                                                    | Silver Iodobromide Emulsion               |                |         |
|                                                    | (average grain size: 0.11 $\mu\text{m}$ ) |                |         |
|                                                    | Gelatin                                   | silver amount: | 1.11 g  |
|                                                    | Coupler C-1                               | silver amount: | 0.04 g  |
|                                                    | Coupler C-2                               | silver amount: | 0.09 g  |
|                                                    | Compound Cpd-A                            | silver amount: | 1.0 mg  |
|                                                    | Compound Cpd-E                            | silver amount: | 0.14 g  |
|                                                    | Compound Cpd-K                            | silver amount: | 2.0 mg  |
|                                                    | Compound Cpd-H                            | silver amount: | 4.4 mg  |
|                                                    | High Boiling Point Organic Solvent Oil-2  | silver amount: | 0.09 g  |
| Fifth Layer: Second Red-Sensitive Emulsion Layer   |                                           |                |         |
| 20                                                 | Emulsion C                                | silver amount: | 0.14 g  |
|                                                    | Emulsion D                                | silver amount: | 0.28 g  |
|                                                    | Gelatin                                   | silver amount: | 0.65 g  |
|                                                    | Coupler C-1                               | silver amount: | 0.05 g  |
|                                                    | Coupler C-2                               | silver amount: | 0.11 g  |
|                                                    | Compound Cpd-E                            | silver amount: | 0.10 g  |
|                                                    | High Boiling Point Organic Solvent Oil-2  | silver amount: | 0.09 g  |
| Sixth Layer: Third Red-Sensitive Emulsion Layer    |                                           |                |         |
| 25                                                 | Emulsion E                                | silver amount: | 0.50 g  |
|                                                    | Gelatin                                   | silver amount: | 1.56 g  |
|                                                    | Coupler C-3                               | silver amount: | 0.63 g  |
|                                                    | Compound Cpd-E                            | silver amount: | 0.11 g  |
|                                                    | Additive P-1                              | silver amount: | 0.16 g  |
|                                                    | High Boiling Point Organic Solvent Oil-2  | silver amount: | 0.04 g  |
| Seventh Layer: Interlayer                          |                                           |                |         |
| 30                                                 | Gelatin                                   | silver amount: | 0.50 g  |
|                                                    | Compound Cpd-D                            | silver amount: | 0.04 g  |
|                                                    | High Boiling Point Organic Solvent Oil-3  | silver amount: | 0.08 g  |
| Eighth Layer: Interlayer                           |                                           |                |         |
| 35                                                 | Yellow Colloidal Silver                   | silver amount: | 0.01 g  |
|                                                    | Gelatin                                   | silver amount: | 1.56 g  |
|                                                    | Compound Cpd-A                            | silver amount: | 0.12 g  |
|                                                    | Compound Cpd-I                            | silver amount: | 0.04 mg |
|                                                    | Compound Cpd-J                            | silver amount: | 0.07 g  |
|                                                    | High Boiling Point Organic Solvent Oil-3  | silver amount: | 0.15 g  |
| Ninth Layer: First Green-Sensitive Emulsion Layer  |                                           |                |         |
| 40                                                 | Emulsion F                                | silver amount: | 0.42 g  |
|                                                    | Emulsion G                                | silver amount: | 0.38 g  |
|                                                    | Emulsion H                                | silver amount: | 0.32 g  |
|                                                    | Surface Fogged Core/Shell Type            | silver amount: | 0.08 g  |
|                                                    | Fine Grain Silver Bromide Emulsion        |                |         |
|                                                    | (average grain size: 0.11 $\mu\text{m}$ ) |                |         |
|                                                    | Gelatin                                   | silver amount: | 1.53 g  |
|                                                    | Coupler C-7                               | silver amount: | 0.07 g  |
|                                                    | Coupler C-8                               | silver amount: | 0.17 g  |
|                                                    | Compound Cpd-B                            | silver amount: | 0.30 mg |
|                                                    | Compound Cpd-C                            | silver amount: | 2.00 mg |
|                                                    | Compound Cpd-K                            | silver amount: | 3.0 mg  |
|                                                    | Polymer Latex P-2                         | silver amount: | 0.02 g  |
|                                                    | High Boiling Point Organic Solvent Oil-2  | silver amount: | 0.10 g  |
| Tenth Layer: Second Green-Sensitive Emulsion Layer |                                           |                |         |
| 45                                                 | Emulsion I                                | silver amount: | 0.16 g  |
|                                                    | Emulsion J                                | silver amount: | 0.34 g  |
|                                                    | Gelatin                                   | silver amount: | 0.75 g  |
|                                                    | Coupler C-4                               | silver amount: | 0.20 g  |
|                                                    | Compound Cpd-B                            | silver amount: | 0.03 g  |

-continued

|                                                      |        |
|------------------------------------------------------|--------|
| Polymer Latex P-2                                    | 0.01 g |
| High Boiling Point Organic Solvent Oil-2             | 0.01 g |
| Eleventh Layer: Third Green-Sensitive Emulsion Layer |        |

|                                          |                |        |
|------------------------------------------|----------------|--------|
| Emulsion K                               | silver amount: | 0.44 g |
| Gelatin                                  |                | 0.91 g |
| Coupler C-4                              |                | 0.34 g |
| Compound Cpd-B                           |                | 0.06 g |
| Polymer Latex P-2                        |                | 0.01 g |
| High Boiling Point Organic Solvent Oil-2 |                | 0.02 g |
| Twelfth Layer: Yellow Filter Layer       |                |        |

|                                                       |                |        |
|-------------------------------------------------------|----------------|--------|
| Yellow Colloidal Silver                               | silver amount: | 0.02 g |
| Gelatin                                               |                | 0.73 g |
| Microcrystal Dispersion of Dye E-1                    |                | 0.24 g |
| Compound Cpd-G                                        |                | 0.02 g |
| Compound Cpd-J                                        |                | 0.04 g |
| High Boiling Point Organic Solvent Oil-3              |                | 0.08 g |
| Thirteenth Layer: First Blue-Sensitive Emulsion Layer |                |        |

|                                                        |                |         |
|--------------------------------------------------------|----------------|---------|
| Emulsion L                                             | silver amount: | 0.35 g  |
| Gelatin                                                |                | 0.55 g  |
| Coupler C-5                                            |                | 0.20 g  |
| Coupler C-6                                            |                | 4.00 g  |
| Coupler C-10                                           |                | 0.02 g  |
| Compound Cpd-E                                         |                | 0.07 g  |
| Compound Cpd-K                                         |                | 0.03 mg |
| Fourteenth Layer: Second Blue-Sensitive Emulsion Layer |                |         |

|                                                      |                |        |
|------------------------------------------------------|----------------|--------|
| Emulsion M                                           | silver amount: | 0.06 g |
| Emulsion N                                           | silver amount: | 0.10 g |
| Gelatin                                              |                | 0.75 g |
| Coupler C-5                                          |                | 0.35 g |
| Coupler C-6                                          |                | 5.00 g |
| Coupler C-10                                         |                | 0.30 g |
| Compound Cpd-E                                       |                | 0.04 g |
| Fifteenth Layer: Third Blue-Sensitive Emulsion Layer |                |        |

|                                                      |                |         |
|------------------------------------------------------|----------------|---------|
| Emulsion O                                           | silver amount: | 0.20 g  |
| Emulsion P                                           | silver amount: | 0.02 g  |
| Gelatin                                              |                | 2.40 g  |
| Coupler C-6                                          |                | 0.09 g  |
| Coupler C-10                                         |                | 0.90 g  |
| Compound Cpd-E                                       |                | 0.09 g  |
| Compound Cpd-M                                       |                | 0.05 mg |
| Fifteenth Layer: Third Blue-Sensitive Emulsion Layer |                |         |

-continued

|                                            |                                                                      |                |
|--------------------------------------------|----------------------------------------------------------------------|----------------|
| 5                                          | High Boiling Point Organic Solvent Oil-2                             | 0.40 g         |
|                                            | Additive P-2                                                         | 0.10 g         |
| Sixteenth Layer: First Protective Layer    |                                                                      |                |
|                                            | Gelatin                                                              | 1.30 g         |
|                                            | Ultraviolet Absorber U-1                                             | 0.10 g         |
|                                            | Ultraviolet Absorber U-2                                             | 0.03 g         |
|                                            | Ultraviolet Absorber U-5                                             | 0.20 g         |
|                                            | Compound Cpd-F                                                       | 0.40 g         |
|                                            | Compound Cpd-J                                                       | 0.06 g         |
|                                            | Dye D-1                                                              | 0.01 g         |
|                                            | Dye D-2                                                              | 0.01 g         |
|                                            | Dye D-3                                                              | 0.01 g         |
|                                            | Dye D-5                                                              | 0.01 g         |
|                                            | High Boiling Point Organic Solvent Oil-2                             | 0.37 g         |
| Seventeenth Layer: Second Protective Layer |                                                                      |                |
|                                            | Fine Grain Silver Iodobromide                                        | silver amount: |
|                                            | Emulsion (average grain size:<br>0.06 $\mu$ m, AgI content: 1 mol %) | 0.05 g         |
|                                            | Gelatin                                                              | 1.80 g         |
|                                            | Compound Cpd-L                                                       | 0.8 mg         |
|                                            | Polymethyl Methacrylate                                              | 5.00 g         |
|                                            | (average particle size: 1.5 $\mu$ m)                                 |                |
|                                            | Copolymer of Methyl Methacrylate/Methacrylic                         | 0.10 g         |
|                                            | Acid in Proportion of 6/4 (average particle                          |                |
|                                            | size: 1.5 $\mu$ m)                                                   |                |
|                                            | Silicone Oil SO-1                                                    | 0.030 g        |
|                                            | Surfactant W-2                                                       | 0.030 g        |

Further, Additives F-1 to F-11 were added to every emulsion layer in addition to the above components. Moreover, Gelatin Hardener H-1 and Surfactants W-1, W-3, W-4, W-5 and W-6 for coating and emulsifying were added to every layer in addition to the above components.

In addition, phenol, 1,2-benzisothiazolin-3-one, 2-phenoxyethanol, phenethyl alcohol, p-hydroxybenzoic acid butyl ester were added as antibacterial and antifungal agents.

Light-sensitive emulsions used in Sample No. 101 are shown in Table 1 below.

TABLE 1

| Emul-<br>sion | Variation                           |                              |                   | Addition<br>( $\times 10^{-4}$ mol/<br>mol-Ag) | Addition<br>( $\times 10^{-4}$ mol/<br>mol-Ag) | Addition<br>( $\times 10^{-4}$ mol/<br>mol-Ag) |       |  |  |  |
|---------------|-------------------------------------|------------------------------|-------------------|------------------------------------------------|------------------------------------------------|------------------------------------------------|-------|--|--|--|
|               | Equivalent-<br>Sphere<br>( $\mu$ m) | Equivalent-<br>Circle<br>(%) | Average<br>Aspect |                                                |                                                |                                                |       |  |  |  |
|               |                                     |                              |                   |                                                |                                                |                                                |       |  |  |  |
| A             | 0.20                                | 16                           | 1.6               | 4.0                                            | S-1                                            | 8.1                                            | S-3   |  |  |  |
| B             | 0.25                                | 15                           | 3.0               | 4.0                                            | S-1                                            | 8.9                                            | S-3   |  |  |  |
| C             | 0.22                                | 14                           | 2.5               | 4.0                                            | S-1                                            | 8.8                                            | S-3   |  |  |  |
| D             | 0.35                                | 10                           | 3.6               | 4.0                                            | S-1                                            | 9.8                                            | S-3   |  |  |  |
| E             | 0.49                                | 16                           | 5.0               | 2.0                                            | S-1                                            | 6.7                                            | S-2   |  |  |  |
| F             | 0.15                                | 15                           | 1.0               | 3.5                                            | S-4                                            | 15.1                                           | III-3 |  |  |  |
| G             | 0.23                                | 14                           | 1.9               | 3.5                                            | S-4                                            | 10.4                                           | III-3 |  |  |  |
| H             | 0.32                                | 11                           | 2.4               | 3.5                                            | S-4                                            | 7.5                                            | III-3 |  |  |  |
| I             | 0.28                                | 11                           | 4.5               | 3.3                                            | S-4                                            | 7.7                                            | III-3 |  |  |  |
| J             | 0.40                                | 16                           | 4.0               | 3.3                                            | S-4                                            | 7.2                                            | III-3 |  |  |  |
| K             | 0.59                                | 20                           | 5.9               | 2.8                                            | S-4                                            | 6.4                                            | III-3 |  |  |  |
| L             | 0.24                                | 14                           | 3.4               | 4.6                                            | S-5                                            | 6.5                                            | S-6   |  |  |  |
| M             | 0.30                                | 10                           | 3.0               | 4.6                                            | S-5                                            | 6.2                                            | S-6   |  |  |  |
| N             | 0.40                                | 9                            | 4.5               | 1.6                                            | S-5                                            | 5.6                                            | S-6   |  |  |  |

TABLE 1-continued

| Emul-<br>sion | Variation<br>Coefficient<br>of                         |                                          | Average<br>Aspect | Sensitizing Dye                 |                              | Sensitizing Dye                                          |      | Sensitizing Dye                                          |      |
|---------------|--------------------------------------------------------|------------------------------------------|-------------------|---------------------------------|------------------------------|----------------------------------------------------------|------|----------------------------------------------------------|------|
|               | Equivalent-<br>Sphere<br>Diameter<br>( $\mu\text{m}$ ) | Equivalent-<br>Circle<br>Diameter<br>(%) |                   | Ratio<br>of<br>Entire<br>Grains | Iodide<br>Content<br>(mol %) | Addition<br>Amount<br>( $\times 10^{-4}$ mol/<br>mol-Ag) | Kind | Addition<br>Amount<br>( $\times 10^{-4}$ mol/<br>mol-Ag) | Kind |
| O             | 0.60                                                   | 15                                       | 5.5               | 1.0                             | S-5                          | 4                                                        | S-6  | 1.5                                                      |      |
| P             | 0.80                                                   | 18                                       | 2.5               | 1.0                             | S-5                          | 3.4                                                      | S-6  | 1.1                                                      |      |

Note 1) All of the above emulsions were silver iodobromide (AgBrI) emulsions chemically sensitized using gold, sulfur and selenium.

Note 2) All of the above emulsions were added with sensitizing dyes before chemical sensitization.

Note 3) Appropriate amounts of Compounds F-5, F-7, F-8, F-9, F-10, F-11, F-12, F-13, F-14 and V-16 were respectively added to the above emulsions.

Note 4) Emulsions A, B, I and J comprise triple structure tabular grains having main planes comprising {100} faces and other emulsions comprise triple structure tabular grains having main planes comprising {111} faces

Note 5) Emulsions A, B, E, F, I and P are emulsions whose internal sensitivities are higher than surface sensitivities.

Note 6) Emulsions E, I and P are emulsions comprising silver chloride grains epitaxially grown after chemical sensitization.

Note 7) Emulsions other than A, E and F comprise grains having 50 or more dislocation lines per one grain observed by a transmission electron microscope.

#### Preparation of Dispersion of Organic Solid Dispersion Dye

Dye E-1 shown below was dispersed according to the following method. That is, water and 70 g of W-4 were added to 1,400 g of a wet cake of the dye containing 30% of water, and stirred to obtain a slurry having 30% dye concentration. Next, 1,700 ml of zirconia beads having an average particle diameter of 0.5 mm were filled in an ultravisco mill (UVM-2) manufactured by Aimex Co., the slurry was passed and the content was pulverized at a

peripheral speed of about 10 m/sec and discharge amount of 0.5 l/min for 8 hours. Beads were removed by filtration and the resulting dispersion was heated at 90° C. for 10 hours for stabilization, then water and gelatin were added to dilute the dispersion to dye concentration of 3%. The average particle size of the obtained fine particles of the dye was 0.4  $\mu\text{m}$  and the extent of distribution of particle sizes [(standard deviation of particle sizes)/(average particle size)  $\times 100$ ] was 18%.

C-1



C-2



35

36

-continued

C-3



C-4



numerals indicate % by weight  
average molecular weight: about 25,000

C-5



C-6



C-7



C-8



-continued

C-9



C-10



Oil-1

Dibutyl Phthalate

Oil-3



Oil-2

Tricresyl Phosphate

Cpd-A



Cpd-B



Cpd-C



Cpd-D



Cpd-E



Cpd-F



Cpd-G



-continued

Cpd-H



Cpd-I



Cpd-K



Cpd-J



Cpd-L



Cpd-M



U-1



U-2



U-3



U-4



U-5



-continued

D-1



D-2



D-3



D-4



D-5



E-1



H-1



-continued

W-1



W-3



W-5



P-1



SO-1



F-1



F-3



F-5



W-2



W-4



W-6



M-1



P-2

Polybutyl acrylate/acrylic acid copolymer in proportion of 95/5

F-2



F-4



F-6



-continued

F-7



F-9



F-11



F-13



S-1



S-2



S-3



S-4



F-8



F-10



F-12



F-14



-continued

S-5



S-6



S-7



S-8



S-9



S-10



## Preparation of Sample Nos. 102 to 116

Sample Nos. 102 to 116 were prepared by replacing Sensitizing Dyes S-4 and III-3 in Emulsions F to K used in Sample No. 101 with equimolar amounts of the dyes as shown in Table 2 below. Further, Sample Nos. 115 and 116 were prepared by not adding Compound VI-16 to each emulsion used in Sample Nos. 101 and 108, respectively. Each piece of the samples thus obtained was subjected to 20 CMS white light exposure for  $\frac{1}{100}$  sec. through a gray wedge, then processed by the following processing step, and sensitometry was carried out. Each of Sample Nos. 101 to 116 subjected to exposure using a halogen lamp of color temperature of 3,200° K. as a light source through a test pattern for RMS value measurement was processed by the following processing step. RMS value of each sample was

obtained by measurement using a micro-densitometer (aperture of measurement: 48  $\mu\text{m}^2$ ).

| Processing Step   | Processing            |                               |                       |                                            |
|-------------------|-----------------------|-------------------------------|-----------------------|--------------------------------------------|
|                   | Processing Time (min) | Processing Temperature (° C.) | Tank Capacity (liter) | Replenish-<br>mg Rate (ml/m <sup>2</sup> ) |
| First Development | 6                     | 38                            | 12                    | 2,200                                      |
| First Washing     | 2                     | 38                            | 4                     | 7,500                                      |
| Reversal          | 2                     | 38                            | 4                     | 1,100                                      |
| Color Development | 6                     | 38                            | 12                    | 2,200                                      |

-continued

|                |   |    |   |       |
|----------------|---|----|---|-------|
| Pre-bleaching  | 2 | 38 | 4 | 1,100 |
| Bleaching      | 6 | 38 | 2 | 220   |
| Fixing         | 4 | 38 | 8 | 1,100 |
| Second Washing | 4 | 38 | 8 | 7,500 |
| Final Rinsing  | 1 | 25 | 2 | 1,100 |

The composition of each processing solution used was as follows.

| First Developing Solution | Tank Solution | Replenisher |
|---------------------------|---------------|-------------|
|---------------------------|---------------|-------------|

|                                                         |          |          |
|---------------------------------------------------------|----------|----------|
| Pentasodium Nitrilo-N,N,N-trimethylenephosphonate       | 1.5 g    | 1.5 g    |
| Pentasodium Diethylenetriaminepentaacetate              | 2.0 g    | 2.0 g    |
| Sodium Sulfite                                          | 30 g     | 30 g     |
| Potassium Hydroquinone-monosulfonate                    | 20 g     | 20 g     |
| Potassium Carbonate                                     | 15 g     | 20 g     |
| Sodium Bicarbonate                                      | 12 g     | 15 g     |
| 1-Phenyl-4-methyl-4-hydroxymethyl-3-pyrazolidone        | 1.5 g    | 2.0 g    |
| Potassium Bromide                                       | 2.5 g    | 1.4 g    |
| Potassium Thiocyanate                                   | 1.2 g    | 1.2 g    |
| Potassium Iodide                                        | 2.0 mg   | —        |
| Diethylene Glycol                                       | 13 g     | 15 g     |
| Water to make                                           | 1,000 ml | 1,000 ml |
| pH (adjusted with sulfuric acid or potassium hydroxide) | 9.60     | 9.60     |

| Reversal Solution                                  | Tank Solution | Replenisher               |
|----------------------------------------------------|---------------|---------------------------|
| Pentasodium Nitrilo-N,N,N-trimethylenephosphonate  | 3.0 g         | same as the tank solution |
| Stannous Chloride Dihydrate                        | 1.0 g         |                           |
| p-Aminophenol                                      | 0.1 g         |                           |
| Sodium Hydroxide                                   | 8 g           |                           |
| Glacial Acetic Acid                                | 15 ml         |                           |
| Water to make                                      | 1,000 ml      |                           |
| pH (adjusted with acetic acid or sodium hydroxide) | 6.00          |                           |

| Color Developing Solution                                                    | Tank Solution | Replenisher |
|------------------------------------------------------------------------------|---------------|-------------|
| Pentasodium Nitrilo-N,N,N-trimethylenephosphonate                            | 2.0 g         | 2.0 g       |
| Sodium Sulfite                                                               | 7.0 g         | 7.0 g       |
| Trisodium Phosphate Dodecahydrate                                            | 36 g          | 36 g        |
| Potassium Bromide                                                            | 1.0 g         | —           |
| Potassium Iodide                                                             | 90 mg         | —           |
| Sodium Hydroxide                                                             | 3.0 g         | 3.0 g       |
| Citrazinic Acid                                                              | 1.5 g         | 1.5 g       |
| N-Ethyl-N-(β-methanesulfonamidoethyl)-3-methyl-4-aminoaniline.Sesquisulfate. | 11 g          | 11 g        |
| Monohydrate                                                                  |               |             |
| 3,6-Dithiaoctane-1,8-diol                                                    | 1.0 g         | 1.0 g       |
| Water to make                                                                | 1,000 ml      | 1,000 ml    |
| pH (adjusted with sulfuric acid or potassium hydroxide)                      | 11.80         | 12.00       |

| Pre-bleaching Solution                             | Tank Solution | Replenisher |
|----------------------------------------------------|---------------|-------------|
| Disodium Ethylenediamine-tetraacetate Dihydrate    | 8.0 g         | 8.0 g       |
| Sodium Sulfite                                     | 6.0 g         | 8.0 g       |
| 1-Thioglycerol                                     | 0.4 g         | 0.4 g       |
| Sodium Bisulfite Addition Products of Formaldehyde | 30 g          | 35 g        |
| Water to make                                      | 1,000 ml      | 1,000 ml    |
| pH (adjusted with acetic acid or sodium hydroxide) | 6.30          | 6.10        |

-continued

| 5                                                       | Bleaching Solution | Tank Solution | Replenisher |
|---------------------------------------------------------|--------------------|---------------|-------------|
| Disodium Ethylenediamine-tetraacetate Dihydrate         | 2.0 g              | 4.0 g         |             |
| Ammonium Ethylenediamine-tetraacetato Ferrate Dihydrate | 120 g              | 240 g         |             |
| Potassium Bromide                                       | 100 g              | 200 g         |             |
| Ammonium Nitrate                                        | 10 g               | 20 g          |             |
| Water to make                                           | 1,000 ml           | 1,000 ml      |             |
| pH (adjusted with nitric acid or sodium hydroxide)      | 5.70               | 5.50          |             |

| 15                                                | Fixing Solution | Tank Solution             | Replenisher |
|---------------------------------------------------|-----------------|---------------------------|-------------|
| Ammonium Thiosulfate                              | 80 g            | same as the tank solution |             |
| Sodium Sulfite                                    | 5.0 g           | same as the tank solution |             |
| Sodium Bisulfite                                  | 5.0 g           | same as the tank solution |             |
| Water to make                                     | 1,000 ml        | same as the tank solution |             |
| pH (adjusted with acetic acid or aqueous ammonia) | 6.60            | same as the tank solution |             |

| 25                                                                           | Final Rinsing Solution | Tank Solution | Replenisher |
|------------------------------------------------------------------------------|------------------------|---------------|-------------|
| 1,2-Benzisothiazolin-3-one                                                   | 0.02 g                 | 0.03 g        |             |
| Polyoxyethylene-p-monononyl-phenyl Ether (average polymerization degree: 10) | 0.3 g                  | 0.3 g         |             |
| Polymaleic Acid (average molecular weight: 2,000)                            | 0.1 g                  | 0.15 g        |             |
| Water to make                                                                | 1,000 ml               | 1,000 ml      |             |
| pH                                                                           | 7.0                    | 7.0           |             |

The results of sensitometry and evaluation of graininess are shown in Table 2 below, GL relative sensitivity was compared based on the relative exposure amount giving the density larger than the minimum density by 1.0. Evaluation of RMS value was conducted as to the value of density 0.7 of the magenta image, which is shown as a relative value taking the value of Sample No. 101 as 100.

TABLE 2

|    | Sample No.        | GL Dye | GL Relative Sensitivity (the larger, the better) | RMS Value (the smaller, the better) |
|----|-------------------|--------|--------------------------------------------------|-------------------------------------|
| 50 | 101 (Comparison)  | S-4    | III-3                                            | 100                                 |
|    | 102 (Comparison)  | S-4    | III-1                                            | 112                                 |
|    | 103 (Comparison)  | S-4    | III-2                                            | 107                                 |
|    | 104 (Comparison)  | S-7    | III-1                                            | 97                                  |
|    | 105 (Comparison)  | S-8    | III-1                                            | 119                                 |
|    | 106 (Invention)   | I-1    | III-1                                            | 129                                 |
|    | 107 (Invention)   | II-1   | III-1                                            | 95                                  |
|    | 108 (Invention)   | II-1   | III-3                                            | 107                                 |
|    | 109 (Invention)   | II-1   | III-1                                            | 84                                  |
|    | 110 (Invention)   | II-2   | V-1                                              | 91                                  |
|    | 111 (Invention)   | II-2   | IV-1                                             | 86                                  |
|    | 112 (Comparison)  | II-1   | S-9                                              | 87                                  |
|    | 113 (Comparison)  | II-2   | S-10                                             | 83                                  |
|    | 114 (Comparison)  | S-4    | S-10                                             | 108                                 |
|    | 115 (Comparison)* | S-4    | III-3                                            | 91                                  |
|    | 116 (Invention)*  | II-1   | III-3                                            | 124                                 |
|    |                   |        | 81                                               | 78                                  |

\*In Sample Nos. 115 and 116, Compound VI-16 was not added to each emulsion.

65 As is apparent from the results in Table 2, a photographic material exhibiting excellent graininess and high sensitivity can be obtained using the compound and the emulsion

51

according to the present invention. It is apparent that high sensitivity and excellent graininess can be compatible for the first time due to the constitution of the present invention.

last time due to the constitution of the present invention.

While the invention has been described in detail and with reference to specific examples thereof, it will be apparent to one skilled in the art that various changes and modifications can be made therein without departing from the spirit and scope thereof.

What is claimed is:

1. A color silver halide photographic material which comprises at least one compound represented by the following formula (I) in a green sensitive silver-halide emulsion layer and at least one sensitizing dye having an absorption maximum in a methanol solution at from 510 to 535 nm in the same green sensitive silver-halide emulsion layer and having a structure represented by the following formula (III), (IV) or (V):



wherein  $R^1$  and  $R^2$  each represents an alkyl group;  $Y$  represents an aryl group or a heterocyclic group;  $V^1$ ,  $V^2$ ,  $V^3$  and  $V^4$  each represents a hydrogen atom, a halogen atom, an alkyl group, an alkoxy group, a hydroxyl group, an alkylthio group, a mercapto group, a cyano group, an acyl group, a carboxyl group, or an alkoxy carbonyl group;  $X^1$  represents a counter ion; and  $m^1$  represents a number of 0 or more necessary for neutralizing a charge in the molecule;



wherein  $R^{31}$  and  $R^{32}$  each represents an alkyl group;  $V^{31}$ ,  $V^{32}$ ,  $V^{33}$ ,  $V^{34}$ ,  $V^{35}$ ,  $V^{36}$ ,  $V^{37}$  and  $V^{38}$  each represents a hydrogen atom or a substituent;  $Z^3$  represents a hydrogen atom, a methyl group or an ethyl group;  $X^3$  represents a counter ion; and  $m^3$  represents a number of 0 or more necessary for neutralizing a charge in the molecule;



wherein  $R^{41}$  and  $R^{42}$  each represents an alkyl group;  $V^{41}$ ,  $V^{42}$ ,  $V^{43}$ ,  $V^{44}$ ,  $V^{45}$ ,  $V^{46}$ ,  $V^{47}$  and  $V^{48}$  each represents a hydrogen atom or a substituent provided that any one of the

52

combinations of  $V^{41}$  and  $V^{42}$ ,  $V^{42}$  and  $V^{43}$ , and  $V^{43}$  and  $V^{44}$  link to each other to form a benzo condensed ring, and any one of the combinations of  $V^{45}$  and  $V^{46}$ ,  $V^{46}$  and  $V^{47}$  and  $V^{47}$  and  $V^{48}$  link to each other to form a benzo condensed ring;  $Z^4$  represents a hydrogen atom, a methyl group or an ethyl group;  $X^4$  represents a counter ion; and  $m^4$  represents a number of 0 or more necessary for neutralizing a charge in the molecule;



wherein  $R^{51}$ ,  $R^{52}$ ,  $R^{53}$  and  $R^{54}$  each represents an alkyl group;  $V^{51}$ ,  $V^{52}$ ,  $V^{53}$ ,  $V^{54}$ ,  $V^{55}$ ,  $V^{56}$ ,  $V^{57}$  and  $V^{58}$  each 25 represents a hydrogen atom or a substituent;  $Z^5$  represents a hydrogen atom a methyl group or an ethyl group;  $X^5$  represents a counter ion; and  $m^5$  represents a number of 0 or more necessary for neutralizing a charge in the molecule.

30 2. The silver halide photographic material as claimed in claim 1, wherein the compound represented by formula (I) is represented by the following formula (II):



wherein R<sup>11</sup> and R<sup>12</sup> each represents an alkyl group; W<sup>1</sup>, W<sup>2</sup>, W<sup>3</sup>, W<sup>4</sup> and W<sup>5</sup> each represents a hydrogen atom or a substituent; V<sup>11</sup> and V<sup>12</sup> each represents a hydrogen atom or 50 a halogen atom; X<sup>2</sup> represents a counter ion; and m<sup>2</sup> represents a number of 0 or more necessary for neutralizing a charge in the molecule.

55 3. The silver halide photographic material as claimed in  
claim 1, which comprises a support having provided thereon  
at least one silver halide emulsion layer, wherein the silver  
halide grains of said silver halide emulsion layer are reduc-  
tion sensitized and said silver halide emulsion layer com-  
60 prises at least one compound represented by formula (I) and  
at least one dye having the absorption maximum in a  
methanol solution at from 510 to 535 nm.

65 4. The silver halide photographic material as claimed in  
claim 3, wherein the compound represented by formula (I)  
is represented by formula (II):



wherein R<sup>11</sup> and R<sup>12</sup> each represents an alkyl group; W<sup>1</sup>, W<sup>2</sup>, W<sup>3</sup>, W<sup>4</sup> and W<sup>5</sup> each represents a hydrogen atom or a substituent; V<sup>11</sup> and V<sup>12</sup> each represents a hydrogen atom or a halogen atom; X<sup>2</sup> represents a counter ion; and m<sup>2</sup> represents a number of 0 or more necessary for neutralizing a charge in the molecule.

5. The silver halide photographic material as claimed in claim 1, wherein the dye having the absorption maximum in a methanol solution at from 510 to 535 nm has the structure represented by formula (III).

6. The silver halide photographic material as claimed in claim 1, which further comprises at least one compound represented by the following formula (VI), (VII) or (VIII):



15 wherein R<sup>101</sup>, R<sup>102</sup> and R<sup>103</sup> each represents an aliphatic group, an aromatic group or a heterocyclic group; M<sup>101</sup> represents a cation; E represents a divalent linking group, and a represents 0 or 1.

\* \* \* \* \*